

Jan. 2, 1945.

W. S. SIMONSON  
CONSTRUCTION METHOD  
Filed Oct. 15, 1942

2,366,156

FIG. 1



FIG. 3



FIG. 2



Wilber S. Simonson Inventor

By

Glen A. Fisch Attorney

## UNITED STATES PATENT OFFICE

2,366,156

## CONSTRUCTION METHOD

Wilber S. Simonson, Spokane, Wash.

Application October 15, 1942, Serial No. 462,164

1 Claim. (Cl. 72—37)

This invention relates to building blocks and a wall formed thereby, it being one object of the invention to provide blocks formed of plastic material and being of such consistency that when a wall is formed of the improved blocks and allowed to dry and harden, it will be substantially a solid wall of set plastic which is fire-proof and moisture-proof.

Another object of the invention is to provide blocks which may be molded just prior to use and built into a wall while still damp, mortar between the blocks being of the same material from which the blocks are formed so that, after the blocks have been built into a wall, the mortar may be troweled and blended into the blocks to provide the wall with a hard and continuous surface which may be covered with a surface coating or painted.

Another object of the invention is to provide building blocks formed of materials easy to obtain and, when mixed, forming a plastic material which may be molded under pressure to the desired shape and form blocks having sufficient strength to withstand heavy bearing pressures.

The invention is illustrated in the accompanying drawing, wherein:

Fig. 1 is a perspective view showing a number of the improved blocks built into a wall.

Fig. 2 is a sectional view taken longitudinally through one of the blocks on the line 2—2 of Fig. 1.

Fig. 3 is a sectional view taken vertically through the wall.

The blocks 1 are formed from a special material and may be of any desired dimensions, it having been found in actual use that blocks 8 x 8 x 16 inches may be easily handled and form a strong wall.

These blocks are formed with passages 2 extending vertically through them and so arranged that when the blocks are built into a wall, the passages register and form air spaces occupying approximately 33% of the bulk of the wall. This provides good insulation for heat and cold and also serves to provide spaces through which water pipes, gas pipes, and electric wiring may pass.

The blocks are formed of a mixture of powdered clay and sulphite waste liquor which may be either raw or in concentrated form. For a block of the dimensions mentioned, forty pounds of dirt containing one pound of powdered clay is used and with this amount of dirt, two pints of raw sulphite liquor are mixed. A block of the proportions set forth will withstand more than twenty-four thousand pounds bearing pressure. When concentrated sulphite waste liquor is used, the block will withstand a test

of forty thousand pounds and, when the blocks are subjected to a pressure of five hundred pounds hydraulic pressure while they are being molded, an increase of 10% is gained over hand-pressed blocks.

The specific quantities set forth are for a block 8 x 8 x 16 inches, and it is to be understood that in quantity production the same proportions will be used. The dirt is the ordinary garden variety which may contain sand and gravel, and the clay and sulphite waste liquor are mixed with it in any desired manner. After the mixture has been formed it is placed in molds and pressed to the desired shape by hand pressure or by power such as hydraulic pressure. The blocks are then removed from the press and built into a wall while still damp. The same material used for making the blocks is used as mortar and the exposed surfaces of the mortar and blocks troweled with a steel trowel to form a smooth surface which is hard as stone when the blocks and mortar have set and are fully dried. The outer surface of the wall is painted with sodium silicate and house paint, as shown at 3 and 4 in Figure 1 of the drawing, to provide a water-proof finish, and the inner surface of the wall may be calsomined or papered.

By placing a substantial concrete footing at the base of the wall and erecting the wall thereon and coating the exterior surface of the wall with a good commercial water-proofing solution, such as asphalt or the like, a basement wall is formed which is dry and free from seepage.

It is to be understood that the blocks may be of any dimensions and shape desired and that for partition walls of a building the air spaces or passages 2 may be omitted. It will also be understood that the plastic material from which the blocks are formed may be molded into a wall, which may be solid, if desired, instead of being formed into blocks to be afterward built into a wall.

Having thus described the invention, what is claimed as new is:

The method of erecting a wall comprising compressing a mass of material consisting of waste sulphite liquor and dirt containing ground clay and forming the same into plastic blocks, placing the newly formed blocks, while still damp, one upon another with mortar of the same material as the blocks between them to form tiers of blocks and interposed mortar, surfaces of the mortar exposed between the blocks being then smoothed and blended into adjoining portions of exposed surfaces of the blocks to form a wall having a hard and substantially unbroken surface when the blocks and mortar are set.

WILBER S. SIMONSON.